

United States Patent [19]  
Sopcak

[11] 3,813,770  
[45] June 4, 1974

[54] METHOD OF ENCAPSULATING COILS  
[75] Inventor: Edward J. Sopcak, Howell, Mich.  
[73] Assignee: Jetro-Matic International Corporation, Denver, Colo.  
[22] Filed: Apr. 19, 1973  
[21] Appl. No.: 352,816

[52] U.S. Cl. 29/605, 29/602, 336/82, 336/84  
[51] Int. Cl. H01f 7/06  
[58] Field of Search 29/602, 605, 608; 336/82, 336/83, 84, 96, 208

[56] References Cited  
UNITED STATES PATENTS  
1,994,534 3/1935 Robinson 29/605

2,419,847 4/1947 Mittermaier 29/608 UX  
2,552,999 5/1951 Pannell et al. 29/605 X

Primary Examiner—Charles W. Lanham  
Assistant Examiner—Carl E. Hall

[57] ABSTRACT

A method of encapsulating conductive coils, including coating the coil with a refractory suspended in a volatilizable organic carrier, heating the coil to volatilize the carrier and leaving a film residue of refractory, and potting the coil in aluminum or the like by pouring molten metal around the coil. The disclosed device includes two copper coils wound in the same direction about common axes and an aluminum body completely encapsulating the coils.

12 Claims, 2 Drawing Figures



PATENTED JUN 4 1974

3,813,770

FIG. 2



FIG. 1



## METHOD OF ENCAPSULATING COILS

## FIELD OF THE INVENTION

The disclosed method is particularly adapted to encapsulating electrically conductive coils in a metal body, wherein the coils may be partially dissolved or washed during casting or potting. The article of manufacture is a magnetic field collecting device, particularly suitable for fuel saving devices.

## SUMMARY OF THE INVENTION

A method of encapsulating conductive coils, such as copper, in aluminum or the like, wherein the coils are first coated with a powdered refractory providing electrical insulation for the coils and preventing washing or dissolving of the coils during potting. The coils are coated with the refractory by first coating the coils with a volatilizable organic carrier having powdered refractory suspended therein and heating the coils to substantially volatilize the carrier and leaving a thin coating of the refractory. The coil is then encapsulated in aluminum by pouring the molten aluminum around the coil and finally cooling the metal, forming an aluminum body.

In the preferred method of this invention, the coils are formed by winding conductive wire around an aluminum arbor or the like. The coils are coated with a powder refractory, such as  $TiO_2$  or  $SiO_2$  suspended in an organic carrier, such as a water soluble acrylic. The coils are placed in a mold on the arbor and the molten aluminum is poured around the coils in the mold, forming the aluminum body integral with the arbor.

The preferred article made by the above process includes two copper coils wound in the same direction about parallel axes and an aluminum body encapsulating the coils. The device is utilized to induce or collect a magnetic field in a fuel saving device and the aluminum body has been found to improve the effectiveness of the device.

## BRIEF DESCRIPTION OF THE DRAWINGS

FIG. 1 is a top perspective view of the mold utilized in the method of this invention with the coils in place; and

FIG. 2 is a top elevation of one embodiment of an article formed by the method of this invention.

## DESCRIPTION OF THE INVENTION

The method of this invention was particularly developed to encapsulate a plurality of conductive coils, such as copper, in insulated relation in a metal body. Such a device is utilized in a new system adapted to improve the engine efficiency of an automotive engine or the like by impressing unidirectional magnetic field across the engine. The disclosed device is retained adjacent a source of pulsating DC current, such as an automotive ignition coil, and a magnetic field is thereby induced in the coils. It has now been discovered that encapsulating the coils in aluminum substantially improves the efficiency of the system, apparently by concentrating or collecting the magnetic field in the coils. The method of this invention is however not limited to this device and has other important applications.

In the disclosed method, the coils are encapsulated in a conventional vertical mold 20 having an internal cavity 22 configured to form the device, as shown in FIG.

1. The coils 24 are supported in spaced relation within the mold cavity on arbors or cylindrical pins 26. The arbors are preferably formed of the same material as the encapsulating material, which in the disclosed embodiment is aluminum. In the preferred embodiment of the engine efficiency system, the disclosed device includes two copper coils wound in the same direction on parallel axes. The coils 24 are left hand windings having copper connectors 28. The connectors in the disclosed embodiment are conventional copper caps used to connect the coils in the engine efficiency system.

The coils in the preferred embodiment are coated with a thin layer of powdered refractory prior to encapsulation. The powdered refractory provides electrical insulation for the coils and prevents surface washing or dissolving of the copper coils by the molten aluminum during encapsulation. The coils are preferably coated with the refractory by first coating the coils with the refractory suspended in a volatilizable organic carrier or binder and then heating the coils to substantially volatilize the carrier, leaving a thin residue of the powdered refractory and sufficient binder to retain the refractory coating. For example, the coils may be dipped in a silicone oil having  $SiO_2$  suspended therein and heated in a conventional furnace to about 500° F. The coils will then have a fine coating of  $SiO_2$  which provides the necessary insulation and protects the coils during encapsulation. The silicone oil may be of commercial grade and the weight percent of silicone is not considered critical.

Another method, which has been found particularly suitable for coating the coils of the disclosed device with a refractory utilizes a commercial acrylic paint which includes titania ( $TiO_2$ ). Titania is used in commercial paint to add opacity. A suitable acrylic paint is a water soluble vinyl acrylic copolymer resin having  $TiO_2$  suspended therein sold by Sears, Roebuck and Company. A typical formulation, by weight, for this paint is as follows:

|                      |       |
|----------------------|-------|
| Titania              | 25.5% |
| Silicates            | 13.3% |
| Vinyl acrylic resins | 14.7% |
| Water                | 46.5% |
| Total                | 100%  |

45 The coils are dipped in the acrylic paint, permitted to dry and then heated in a conventional furnace at a temperature of between about 500° and 550° F. until the acrylic resin is substantially volatilized. The coils then include a thin coating of titania. It has also been found that other refractories may also be utilized, including  $Al_2O_3$ ,  $MgO$ ,  $ZrO_2$  and mullite, which is  $Al_2O_3 \cdot SiO_2$ .

50 As described above, the coils 24 are supported within the mold cavity 22 on aluminum arbors 26. The ends of the arbors may be received in holes in the bottom of the mold, not shown, which support the arbors. The molten aluminum is then poured around the coils, forming an integral aluminum body 30, as shown in FIG. 2. The aluminum arbors are then integral with the and the copper connectors 28 provide contact to the encapsulated coils 24. In the disclosed embodiment, the body 30 is generally rectangular with a concave face 32 which is secured to a cylindrical supporting surface in the engine efficiency system, such as an automotive ignition coil. In this location, the ignition coil is a source of pulsating DC current, inducing a current and magnetic field in the coils 24. It has now been discovered that the aluminum body 30 substantially im-

proves the efficiency of the system, apparently because the aluminum body collects or concentrates the electric field. In the engine efficiency system, the coils must be isolated electrically and insulated from the engine and system. The powdered refractory provides the necessary insulation and prevents surface washing of the copper during encapsulation.

As described above, the method of this invention is not limited to the specific materials. The preferred embodiment of the device includes copper coils encapsulated in an aluminum body. A suitable material for the coils is an uncoated bus bar wire, which is commercially pure copper. Copper melts at 1,981° F., which is above the melting temperature of aluminum. A suitable material for the body is commercial 319 aluminum, which includes 4 percent by weight copper and 6 percent by weight silicon. The aluminum melts at between 1,050° and 1,075° F. and the normal pouring temperature of commercial 319 aluminum is 1,350° F. At these temperatures, however, the molten aluminum would wash the surface of the copper wires, partially dissolving the copper and possibly breaking electrical contact. The coating of the wires with a powdered refractory then protects the coils and provides the necessary electrical insulation.

I claim:

1. A method of encapsulating a copper coil in an aluminum body, comprising:

- a. coating a copper coil with a refractory powder suspended in a substantially volatilizable fluid organic carrier,
- b. heating the coil to volatilize said organic carrier, above the volatilization temperature of said fluid organic carrier, but below the melting temperature of said copper coil, leaving a residue of said refractory powder on said coil,
- c. potting said coil coated with said powdered refractory in aluminum by pouring molten aluminum around said coil, and
- d. cooling the aluminum, thereby forming an aluminum body encapsulating said coil.

2. The method defined in claim 1, including coiling a copper wire around an aluminum arbor, thereby forming said copper coil.

3. The method defined in claim 1, wherein said liquid organic carrier is a commercial acrylic paint having powdered  $TiO_2$  suspended therein, including dipping said coil in said acrylic paint and heating said coated coil to a temperature between about 500° and 550° F., thereby volatilizing the acrylic binder and leaving a thin coating of powdered  $TiO_2$ .

4. The method defined in claim 1, characterized in that said organic carrier is a silicone oil having powdered  $SiO_2$  suspended therein, including heating said coil to a temperature above about 500° F., thereby volatilizing said oil and leaving a residue of  $SiO_2$  on said coil.

5. The method defined in claim 1, including inserting said coil coated with said refractory in a mold having the preferred internal configuration and pouring molten aluminum into said mold, wherein said refractory prevents washing of the copper coil.

6. A method of encapsulating a plurality of conductive coils in aluminum, said coils having a melting temperature above the melting temperature of aluminum and electrically insulated from each other, comprising the steps of:

10 a. coiling conductive wire around two aluminum arbors thereby forming two separate conductive coils, one on each of said arbors,

b. coating each of said coils with a thin layer of powdered refractory,

c. inserting said coils, while still on said arbors, into a mold in spaced relation,

d. pouring molten aluminum into said mold, around said coils, wherein said refractory prevents washing of the coils, and

e. cooling said aluminum, thereby forming an aluminum article having conductive coils encapsulated therein.

20 7. The method defined in claim 6, wherein said conductive coils are each coated with a refractory selected from the group consisting of  $SiO_2$ ,  $TiO_2$ ,  $Al_2O_3$ ,  $MgO$ ,  $SrO_2$  and mullite, by coating said coils with said refractory suspended in a liquid organic carrier which is substantially volatilizable at elevated temperatures and heating said coils above the volatilization temperature of the binder, but below the melting temperature of aluminum.

25 8. The method defined in claim 7, wherein said organic binder is a water soluble acrylic and said coils are heated to a temperature above about 500° F.

9. The method defined in claim 8, wherein said acrylic binder is a commercial paint having powdered  $TiO_2$  suspended therein, including heating said coils to a temperature between about 500° and 550° F., leaving a residue of powdered  $TiO_2$  on said coils.

10. The method defined in claim 7, wherein said organic carrier is a silicone oil having  $SiO_2$  suspended therein, including heating said coils above about 500° F.

11. A method of encapsulating a plurality of conductive coils in a conductive metal having a melting temperature below the melting temperature of said coils and said coils electrically insulated from each other, comprising the steps of:

a. coiling conductive wire around two cylindrical arbors, thereby forming two separate conductive coils, one on each of said arbors,

b. coating each of said coils with a thin layer of powdered refractory by first coating said coils with a refractory suspended in a volatilizable carrier and heating said coils to volatilize said carrier, leaving a residue coating of said refractory,

c. inserting said coils, while still on said arbors, into a mold in spaced relation,

d. pouring said metal in a molten state into said mold, around said coils, wherein said refractory prevents washing of said coils, and

e. cooling said metal, thereby forming a metal article having conductive coils encapsulated therein.

12. The method defined in claim 11, wherein said metal is aluminum and said coils are copper, including pouring said aluminum at about 1350° F.

\* \* \* \* \*